# EUROPEAN PATENT APPLICATION

(11) **EP 4 707 433 A1**
(43) Date of publication of application: **11.03.2026**
(21) Application number: 24936687.3
(22) Date of filing: 11.11.2024
(51) Int. Cl.: C25D 11/22, C25D 11/04, C25D 11/30, C25D 11/26

(54) **RARE EARTH-BASED ELECTROLYTIC COLORING METHOD AND ALLOY PRODUCT**

(30) Priority: 25.04.2024 CN 202410507867
(71) Applicant: Shenzhen Xin Mao Xin Industrial Co., Ltd., Shenzhen, Guangdong 518000 (CN)
(72) Inventor: LIU, Qiuhua, Shenzhen, Guangdong 518000 (CN); ZHANG, Huailiang, Shenzhen, Guangdong 518000 (CN); ZHENG, Hekai, Shenzhen, Guangdong 518000 (CN)
(74) Representative: Metida
(86) International application number: PCT/CN2024/131169
(87) International publication number: WO 2025/222795

(57) **Abstract**

A rare earth-based electrolytic coloring method and an alloy product therefrom are provided in the disclosure. The method includes: quickly raising a voltage after the workpiece in the electrolyte is anodized to form an oxide film, and taking a constant voltage mode so that the oxide film is broken down, melted, sintered and re-formed under conditions of a high frequency, a high voltage and instantaneous high temperature, so as to generate a ceramic film layer metallurgically combined with a substrate after multiple cycles. The oxide film is thicker and is with lower reflectivity and an appearance as a matte black anode, and has good color consistency and no chromatic aberration. The electrolyte includes sodium silicate with a concentration of 5 to 70 g/L, sodium tungstate with a concentration of 1 to 18 g/L, disodium edetate with a concentration of 2 to 10 g/L and rare earth salt with a concentration of 1 to 2 g/L.

## Description

### TECHNICAL FIELD

The disclosure relates to the technical field of surface treatment, in particular to a rare earth-based electrolytic coloring method, an electrolyte, and an alloy product.

### BACKGROUND ART

Electrolytic coloring, also known as plasma electrolytic oxidation, is developed from anodic oxidation technology. The electrolytic coloring is a surface treatment technology, and a workpiece to be processed can be electrolytically colored with a micro-arc oxidation process, so that the workpiece can be endowed with various colors and decorative effects. A metal surface processed with existing surface treatment processes has defects of a thin oxide film and high reflectivity.

### SUMMARY

The disclosure provides an electrolytic coloring electrolyte and method for metals and alloys, a product of metals and alloys, which can increase a thickness of a ceramic film layer on a metal surface and reduce reflectivity.

In a first aspect, a rare earth-based electrolytic coloring method is provided in the disclosure, which is applied to magnesium alloy, titanium alloy or aluminum alloy, and includes:
placing a workpiece into an electrolytic cell to form a fine and uniform oxide film on a surface of the workpiece after electrifying;
keeping the workpiece in the electrolytic cell for electrolytic coloring treatment, and generating a ceramic film layer metallurgically combined with a substrate after the oxide film is broken down, melted, sintered and re-formed; during the electrolytic coloring treatment, a voltage being rapidly increased to a preset high voltage and then a thickness of the ceramic film layer being rapidly increased in a high-frequency constant voltage mode;
washing the electrolytic colored workpiece with water, the washing with water referring to cleaning the workpiece using deionized water at a room temperature of 25°C;
washing the water-washed workpiece with warm water; and
air-drying and baking the workpiece subjected to the washing with warm water.

An electrolyte consists of 5 to 70 g/L of sodium silicate, 3 to 30 g/L of potassium hydroxide, 3 to 18 g/L of potassium fluoride, 5 to 25 g/L of sodium fluoride, 1 to 18 g/L of sodium tungstate, 5 to 25 g/L of ammonium metavanadate, 2 to 10 g/L of disodium edetate, 1 to 9 g/L of triethanolamine, 1 to 18 g/L of potassium ferricyanide, 3 to 13 g/L of sodium tetraborate, 5 to 15 g/L of glycerol, 2 to 15 g/L of sodium carbonate, 3 to 10 g/L of hexamethylene tetramine, and 1 to 2 g/L of rare earth salt.

In some embodiment, the rare earth salt includes a mixture of one or more of cerium nitrate, lanthanum nitrate and dysprosium nitrate and one or more of yttrium nitrate, erbium nitrate and thulium nitrate.

In some embodiments, during electrolysis, a bidirectional asymmetric pulse power supply is used, with a frequency of 500 Hz to 1200 Hz and a duty cycle of 10% to 25%.

In some embodiments, the electrolyte is with a temperature of 250°C to 400°C and a duration of 20 minutes to 30 minutes.

In a second aspect, an alloy product from rare earth-based electrolytic coloring is provided in the disclosure, which is prepared by the electrolytic coloring method described in the first aspect.

In some embodiments, surface reflectivity of the product is less than 5%, and a surface oxide film thickness is 15 to 100 um.

In some embodiments, surface reflectivity of the product for laser with a wavelength of 1550 nm is 3.62% to 4.98%; and surface reflectivity of the product for laser with a wavelength of 905 nm is 1.6% to 2.3%.

In some embodiments, the metal alloy includes magnesium alloy, titanium alloy or aluminum alloy.

According to above embodiments, after the workpiece in the electrolyte is anodized to form the oxide film, the voltage is quickly raised, and the oxide film is broken down, melted, sintered and re-formed under a constant voltage mode with a high frequency and a high voltage, so as to generate the ceramic film layer metallurgically combined with the substrate after multiple cycles. As the sodium silicate, the sodium tungstate, the disodium edetate and the rare earth salt are added to the electrolyte, the oxide film is thicker and is with lower reflectivity and an appearance as a matte black anode, has good color consistency, no chromatic aberration, and exhibits properties such as corrosion resistance and wear resistance.

### BRIEF DESCRIPTION OF THE DRAWINGS

FIG. 1 is a schematic view of a scanning electron microscopic image of a ceramic layer according to an embodiment;
FIG. 2 is a partial enlarged view of FIG. 1;
FIG. 3 is a schematic topography of a section of a ceramic layer according to an embodiment;
FIG. 4(a) is a schematic view showing influence of different voltages on a film thickness in a constant voltage mode according to an embodiment;
FIG. 4(b) shows surface morphology of a film layer in a constant voltage mode of 300 V according to an embodiment;
FIG. 4(c) shows surface morphology of a film layer in a constant voltage mode of 400 V according to an embodiment; and
FIG. 4(d) shows surface morphology of a film layer in a constant voltage mode of 440 V according to an embodiment.

### DETAILED DESCRIPTION

The present disclosure will be further described in detail below through specific embodiments in connection with attached drawings. Like elements in different embodiments have been given associated like element numbers. In following embodiments, many details are described in order to make the disclosure be better understood. However, those skilled in the art can easily realize that some of features can be omitted in different situations or can be replaced with other elements, materials and methods. In some cases, some operations related to this disclosure are not shown or described in the specification, in order to avoid a core part of this disclosure being overwhelmed by excessive description. For those skilled in the art, it is not necessary to describe these related operations in detail, and they can fully understand related operations according to description in the specification and general technical knowledge in this art.

An electrolytic coloring method of metal alloy is provided in the disclosure, which includes following steps.

First, the workpiece is ultrasonically cleaned, that is, the workpiece is placed in a container, an acetone solution with a mass concentration of more than 99% is added, and the workpiece is ultrasonically cleaned in an ultrasonic cleaning machine.

Then, the workpiece is placed into an electrolytic cell to form a fine and uniform oxide film on a surface of the workpiece after electrifying (this process is similar to anodic oxidation with an alkaline electrolyte).

The workpiece is kept in the electrolytic cell for electrolytic coloring treatment, and a ceramic film layer metallurgically combined with a substrate is generated after the oxide film is broken down, melted, sintered and re-formed; and during the electrolytic coloring treatment, a voltage is rapidly increased to a preset high voltage (for example, 300 V~440 V) and then a thickness of the ceramic film layer is rapidly increased in a constant voltage mode (see FIG. 4 (b) ~ 4 (d) for surface morphology of the film layer under different constant voltages).

The electrolytic colored workpiece is washed with water.

The water-washed workpiece is washed with warm water.

The workpiece subjected to the washing with warm water is air-dried and baked.

An electrolyte consists of 5 to 70 g/L of sodium silicate, 3 to 30 g/L of potassium hydroxide, 3 to 18 g/L of potassium fluoride, 5 to 25 g/L of sodium fluoride, 1 to 18 g/L of sodium tungstate, 5 to 25 g/L of ammonium metavanadate, 2 to 10 g/L of disodium edetate, 1 to 9 g/L of triethanolamine, 1 to 18 g/L of potassium ferricyanide, 3 to 13 g/L of sodium tetraborate, 5 to 15 g/L of glycerol, 2 to 15 g/L of sodium carbonate, 3 to 10 g/L of hexamethylene tetramine, and 1 to 2 g/L of rare earth salt. The rare earth salt includes a mixture of one or more of cerium nitrate, lanthanum nitrate and dysprosium nitrate and one or more of yttrium nitrate, neodymium nitrate and thulium nitrate.

In a specific embodiment, during electrolysis, a bidirectional asymmetric pulse power supply is used, with a frequency of 500 Hz to 1200 Hz and a duty cycle of 10% to 25%. The electrolyte is with a temperature of 250°C to 400°C and a duration of 20 minutes to 30 minutes. The electrolysis duration starts from time when the workpiece is placed into the electrolytic cell for electrifying until the electrolytic coloring is completed. The workpiece subjected to the electrolytic coloring is taken out and washed with water.

It should be particularly noted that, in general, the high-frequency power supply may increase a growth rate of the oxide film, but result in a relatively small thickness of the film, and an excessively high voltage may cause local breakdown of the oxide film, which is not conducive to corrosion resistance of the oxide film.

Therefore, the sodium silicate is selected as a main salt of the electrolyte in this disclosure, which facilitates generation of a complete micro-arc oxidation film with plane continuity on a surface of the substrate, which can improve compactness of the film, and existence of the sodium silicate can reduce a corrosion current density of the oxide film and significantly improve the corrosion resistance of the film. The sodium silicate can increase conductivity of the electrolyte, thus reducing an arcing voltage on the surface of the substrate, causing a more efficient oxidation process and a larger film formation speed during the electrolytic coloring. Moreover, because the sodium tungstate and the disodium edetate are added to the electrolyte, they can improve conductivity and stability of the electrolyte, thus contributing to formation of a uniform and dense oxide film.

In addition, because rare earth elements contain both heavy rare earth and light rare earth, a new phase is generated on a surface of the product, and its structure is refined and is more uniform and dense, thus reducing the surface reflectivity of the product. The lanthanum nitrate (La(NO3)3) can promote formation of the oxide film and improve its compactness and hardness. Rare earth elements such as cerium (Ce) and yttrium (Y) can be added to an electrolyte for micro-arc oxidation to improve a formation speed of the oxide film. A micro-arc oxidation film of magnesium alloy obtained by treating with a rare earth neodymium (Nd) salt solution for a short time can be with a uniform thickness distribution.

It can be seen that the electrolyte in this disclosure includes sodium silicate with a concentration of 5 to 70 g/L, sodium tungstate with a concentration of 1 to 18 g/L, disodium edetate with a concentration of 2 to 10 g/L and rare earth salt with a concentration of 1 to 2 g/L, thus reducing holes and cracks in the film layer, improving the compactness, and thus reducing the surface reflectivity of the product. Advantages of rapid film formation by a high-frequency power supply and rapid electrolytic coloring by a high-voltage power supply are fully exerted, and defects that a thickness of the formed film by the high-frequency power supply is relatively thin and an overhigh voltage is not good to the corrosion resistance of the oxide film are overcome.

As shown in FIGS. 1 to 3 and 4 (a) to 4 (d), at the constant voltage mode of a high frequency and a high voltage, the ceramic film layer can be obtained quickly in the disclosure, and the thickness of the ceramic film layer is relatively thick. For example, in an example of FIG. 3, the ceramic film layer is with a dense layer of 9 um and a porous layer of 12 um, and is 21 um in total, which makes the surface reflectivity of the product low.

In this disclosure, under action of the high frequency power supply, the oxide film is rapidly formed and continuously thickened, a number of micropores in the oxide film is reduced, and the micropores becomes larger in pore size and melting occurs; and after melting, the oxide film solidifies to form small particles, which cover part of the micropores and further reduce the number of micropores. Under action of the high voltage power supply, the oxide film is repeatedly broken down at many positions thereon, and the molten oxide is sprayed around from the micropores and repeatedly accumulated, after which the molten oxide solidifies into a hard ceramic layer under action of liquid quenching of the electrolyte. Meanwhile, the high voltage power supply causes non-ferrous metal ions in the electrolyte to penetrate into the oxide film to realize coloring, thus enhancing coloring depth and durability.

In a third aspect, an alloy product from rare earth-based electrolytic coloring is provided in the disclosure, which is prepared by the electrolytic coloring method described in the first aspect.

In some embodiments, surface reflectivity of the product is less than 5%, and a surface oxide film thickness is 15 to 100 um.

In some embodiments, surface reflectivity of the product for laser with a wavelength of 1550 nm is 3.62% to 4.98%; and surface reflectivity of the product for laser with a wavelength of 905 nm is 1.6% to 2.3%.

In some embodiments, the metal alloy includes magnesium alloy, titanium alloy or aluminum alloy.

Perception ability of a lidar is very important for driving safety of autonomous driving, and low reflectivity of products is essential. In a specific embodiment, in order to be applied to appearance treatment of the lidar and an onboard optical structural parts, aluminum alloy is used as an anode and stainless steel is used as a cathode, and the oxide film is formed on the workpiece in the electrolyte under action of an electric field, and the oxide film is broken down, melted, sintered and re-formed under conditions of a high voltage and instantaneous high temperature, which is repeated for many times so as to generate a ceramic film metallurgically combined with the substrate, and thus the oxide film is thicker and is lower in reflectivity. The aluminum alloy includes: AL6061 aluminum profile, ADC12, HTCO2 and ENAC43500 die-casting aluminum.

Through diffuse reflection test, the surface reflectivity of the product in this disclosure is obtained to be less than 5%, with good low reflectivity performance.

In a specific embodiment, measured results with a R1000 reflectivity tester from Yuke Instruments Co.,Ltd. show that surface reflectivity of the product for laser with a wavelength of 1550 nm is 3.62% to 4.98%; and surface reflectivity of the product for laser with a wavelength of 500 nm/850 nm/905 nm is 1.6% to 2.5%.

Compared with other existing surface treatment processes, a thickness of the surface oxide film of the electrolytic colored product from the disclosure is 15 to 100 um, which realizes properties such as low reflection, corrosion resistance, wear resistance, high insulation performance, high hardness, and low friction coefficient.

In addition, features, operations or characteristics described in the specification can be combined in any suitable way to form various embodiments. Meanwhile, steps or actions in the method description can also be exchanged or adjusted in order in a way obvious to those skilled in the art.

Above examples are used to illustrate the disclosure, which is only intended to help understand the disclosure, but not limit the disclosure. For those skilled in the art to which the present disclosure belongs, several simple deduction, variation or substitution can be made according to an idea of the present disclosure.

## Claims

1. A rare earth-based electrolytic coloring method, which is applied to magnesium alloy, titanium alloy or aluminum alloy, and comprises:
placing a workpiece into an electrolytic cell to form a fine and uniform oxide film on a surface of the workpiece after electrifying;
keeping the workpiece in the electrolytic cell for electrolytic coloring treatment, and generating a ceramic film layer metallurgically combined with a substrate after the oxide film is broken down, melted, sintered and re-formed; during the electrolytic coloring treatment, a voltage being rapidly increased to a preset high voltage and then a thickness of the ceramic film layer being rapidly increased in a high-frequency constant voltage mode;
washing the electrolytic colored workpiece with water;
washing the water-washed workpiece with warm water; and
air-drying and baking the workpiece subjected to the washing with warm water; wherein.

2. an electrolyte consists of 5 to 70 g/L of sodium silicate, 3 to 30 g/L of potassium hydroxide, 3 to 18 g/L of potassium fluoride, 5 to 25 g/L of sodium fluoride, 1 to 18 g/L of sodium tungstate, 5 to 25 g/L of ammonium metavanadate, 2 to 10 g/L of disodium edetate, 1 to 9 g/L of triethanolamine, 1 to 18 g/L of potassium ferricyanide, 3 to 13 g/L of sodium tetraborate, 5 to 15 g/L of glycerol, 2 to 15 g/L of sodium carbonate, 3 to 10 g/L of hexamethylene tetramine, and 1 to 2 g/L of rare earth salt.

3. The electrolytic coloring method according to claim 1, wherein the rare earth salt comprises a mixture of one or more of cerium nitrate, lanthanum nitrate and dysprosium nitrate and one or more of yttrium nitrate, neodymium nitrate and thulium nitrate.

4. The electrolytic coloring method according to claim 1 or 2, wherein during electrolysis, a bidirectional asymmetric pulse power supply is used, with a frequency of 500 Hz to 1200 Hz and a duty cycle of 10% to 25%.

5. The electrolytic coloring method according to claim 1, wherein the electrolyte is with a temperature of 250°C to 400°C and a duration of 20 minutes to 30 minutes.

6. An alloy product from rare earth-based electrolytic coloring, which is prepared by the electrolytic coloring method according to any one of claims 1 to 4.

7. The alloy product from rare earth-based electrolytic coloring according to claim 5, wherein surface reflectivity of the product is less than 5%, and a surface oxide film thickness is 15 to 100 um.

8. The alloy product from rare earth-based electrolytic coloring according to claim 6, wherein surface reflectivity of the product for laser with a wavelength of 1550 nm is 3.62% to 4.98%; and surface reflectivity of the product for laser with a wavelength of 905 nm is 1.6% to 2.3%.

9. The alloy product from rare earth-based electrolytic coloring according to any one of claims 5 to 7, wherein the metal alloy comprises magnesium alloy, titanium alloy or aluminum alloy.

## Amended claims

### Amended claims under Art. 19.1 PCT

1. A method of electrolytic coloring based on rare earth, **characterized in that** it is applied to magnesium alloy and titanium alloy. Gold or aluminum alloy, including:
The workpiece is put into the electrolytic tank, and a fine and uniform oxide film is formed on the surface of the workpiece after the electric current is applied.
The workpiece is kept in the electrolytic cell for electrolytic coloring treatment, and the oxide film is broken down, melted and burned. After the film is formed and reformed, a ceramic film layer metallurgically bonded to the substrate is generated; during the electrolytic coloring process,
The voltage is rapidly increased to the preset high voltage, and then the thickness of the ceramic film layer is quickly increase;
The workpiece after electrolytic coloring is washed with water; The workpiece is washed with warm water after washing.
The workpiece was dried and baked after washing with warm water.
The composition of the electrolyte is as follows: sodium silicate 5-70g/L, potassium hydroxide 3-30g/L, potassium fluoride.Format:Indent:Left:0mm,First-line indent:2 characters, Tab position: 3-18 g/L, sodium fluoride 5-25 g/L, sodium tungstate 1-18 g/L, ammonium metavanadate 5-25 g/L, ethylenediaminetetraacetic acid not 2.79 characters, no items or numbers Sodium dihydrogen phosphate 2-10g/L, triethanolamine 1-9g/L, potassium ferricyanide 1-18g/L, sodium tetraborate 3-13g/L, glycerol 5-15g/L sodium carbonate, 3-10g/L hexamethylenetetramine, 1-2g/L rare earth salt.

2. The rare earth salts include:
One or more of cerium nitrate, lanthanum nitrate, and dysprosium nitrate combined with one or more of yttrium nitrate, neodymium nitrate, and thulium nitrate of the mixture.

3. The electrolytic coloring method according to claim 1, **characterized in that**, during electrolysis, bidirectional non-deletion is adopted:or 2 The pulse power supply is symmetrical, the frequency is 500Hz-1200Hz, the duty cycle is 10%-25%.

4. The electrolytic coloring method as claimed in claim 1, wherein the electrolyte temperature is The temperature was 25°C-40°C, and the electrolysis time was 20-30 minutes.

5. A rare earth-based electrolytic coloring alloy product, **characterized in that** the product utilizes root The electrolytic coloring method is prepared according to claim 1.

6. The electrolytically colored alloy product as claimed in claim 5, **characterized in that** the product The surface reflectivity is less than 5% and the oxide film thickness is 15~ 100um.

7. The electrolytically colored alloy product as claimed in claim 6, **characterized in that** the product is The surface reflectivity of the 1550nm laser ranges from 3.62% to 4.98%, and the product exhibits reflectivity at 905nm. The surface reflectivity of the laser is 1.6% to 2.3%.
